

Oct. 10, 1961

K. MEYER ET AL

3,003,863

SINTERING OF ENDOOTHERMIC MATERIALS

Filed Oct. 23, 1958

Fig. 1



Fig. 1a



Fig. 2a

Inventors:

KURT MEYER

HANS RAUSCH

By  
Bailey, Stephen & Huettig  
ATTORNEYS

# United States Patent Office

3,003,863

Patented Oct. 10, 1961

1

3,003,863

**SINTERING OF ENDOOTHERMIC MATERIALS**  
Kurt Meyer, Frankfurt am Main, and Hans Rausch,  
Oberursel (Taunus), Germany, assignors to Metallge-  
sellschaft Aktiengesellschaft, Frankfurt am Main, Ger-  
many

Filed Oct. 23, 1958, Ser. No. 769,128

Claims priority, application Germany Nov. 5, 1957  
1 Claim. (Cl. 75—5)

This invention relates to sintering and, in particular, to the sintering of endothermic materials.

In the sintering of endothermic materials on a sinter grate or band, as in the sintering of iron ores, it is known to supply the heat by the simultaneous use of solid fuels and hot gases. Moreover, it has been established that with the use of mixed solid and gaseous fuels the fuel efficiency is greater than that obtained with the use of solid fuels only and that the fuel efficiency in using gases alone is much lower than with the use of solid fuel alone.

Generally in sintering processes, especially at the sintering of iron ores, a melting zone is formed in the sinter bed. In this zone there is the sinter mixture in a doughy condition which is necessary to bring the material to be sintered in the desired condition. Because of its doughy condition the melting zone has a certain resistance to the gases to be drawn through. The resistance is the greater the thicker the melting zone is. Therefore it is desired to keep the melting zone not greater than necessary so that the gas passage is not restrained too much. A great gas passage is desired to promote the combustion and the other processes in the sinter bed and thereby to result a rather great efficiency and production of the sinter apparatus.

The object of this invention is to obtain a greater efficiency in the use of gaseous fuel in the heat treatment of endothermic materials.

It has been discovered in this invention that in a bed of endothermic material mixed with solid fuel and with simultaneous use of gaseous fuel and which is burned on a sinter band the decrease in the efficiency of the use of gaseous fuels has, for one of its reasons, the fact that during the burning of the solid fuel together with the heat from the hot gases the melting zone is increased. The hot gases tend to make the melting zone of greater thickness than would occur in the use of solid fuel alone, and this zone of greater thickness stops the passage of the hot gases through the bed and thus also slows the sinter process and the velocity of the sinter band, and the sinter production is decreased. Thus the efficiency of the sinter band is reduced. The reason for this fact is that in the first part of the sinter process hot gases containing oxygen are led to the sinter bed instead of the cool air which is usually drawn through.

According to this invention, the extent of the thickness of this melting zone is kept as thin as possible by subjecting the bed of material to hot gases of successively varying temperatures. Preferably, immediately after feeding the sinter band with the sinter mixture, hot gases at about 1000° C. are drawn through the bed in order to ignite the solid fuel in the bed. Immediately thereafter, gas at a lower temperature is drawn through the bed in order to create in the sinter bed above the melting a zone of somewhat lower temperature. If desirable, by using several times alternatively of higher and lower temperatures, various successive layers of various temperature can be created in series.

The result is that an excessive thickness of the melting zone is not caused by the drawing of hot gases through the sinter bed with the simultaneous burning of the solid fuel in the bed and thus the production of the sinter

2

band is not reduced. On the other hand it can be insured that, by the suitable regulating of the temperatures of the hot gases in the various parts of the hood such a quantity of calories are brought therein, that a considerable part of the entire heat requirement for the sintering bed will be supplied by the hot gases drawn through the sinter bed.

The means by which the objects of the invention are obtained are described more fully with reference to the accompanying drawings, in which:

FIGURE 1 is a schematic cross-sectional view of a sinter apparatus according to the prior art;

FIGURE 1a is a detail view of the sinter bed exaggerated in vertical scale;

FIGURE 2 is a schematic cross-sectional view of a sinter apparatus according to this invention; and

FIGURE 2a is an enlarged detail view of FIGURE 2 exaggerated in vertical scale.

The sinter apparatus has a continuous grate or band 1 upon which is placed a protective layer of material 2. The material to be sintered is formed as a bed 3 upon layer 2. The gas for igniting the solid fuel in bed 3 is drawn from hood 4 through the sinter bed. Additional hot gases are supplied through hoods 5 and 6.

As an example of this invention, the bed 3 is composed of 40 parts recycled pyrites, 10 parts blast furnace dust, 20 parts magnetite concentrates, 8 parts pelletized mill dust, 22 parts purple ferric oxide ore, 25 parts recycled material and 7.5 parts coke fines. Hot gas at a temperature of about 1000° C. is drawn through the bed 3 from the hood 4. If the gas supplied from hoods 5 and 6 were at the same temperature as the gas from hood 4, then a melting zone *a* would be formed in bed 3. However, according to this invention, a gas at a lower temperature, such as 800° C., is drawn through the bed from hood 5 and, as shown in FIGURES 2 and 2a, the melting zone *b* is formed of less thickness than zone *a* of FIGURE 1a. A hotter gas having a temperature higher of that in hood 5, such as 900° C., is drawn from hood 6 through bed 3 and forms a zone *c* as a layer overlying zone *b*. This zone *c* has a temperature less than that of the melting temperature in zone *b*, but allows sufficient heat to be drawn through the bed to maintain melting zone *b*.

The temperatures given in the above example can be raised or lowered depending upon the particular characteristics of the raw material being heat treated. The heat supplied by the hot gases should not be great enough to increase the width of melting zone *b*. The temperatures of the gases drawn from the hood following the first ignition hood are kept as high as possible but below the point which would cause a widening of the melting zone.

## EXAMPLE 1

### Conventional sintering

On a sinter machine with a sintering area of 75 m.<sup>2</sup> (2.50 meter width, 30 meter length) a steel iron sinter mixture was sintered. The composition of the sinter mixture was as follows:

Parts

|                                                                                 |     |
|---------------------------------------------------------------------------------|-----|
| Ore with a moisture content of 8 percent and a loss on ignition of 11.3 percent | 100 |
| Recycled material                                                               | 32  |
| Coke fines                                                                      | 8.3 |
| With a heating value of 5200 calories per kg.                                   |     |

The sinter mixture was charged onto the sinter band with a height of layer of 28 cm. including a grate protective layer of 2 cm. After the charging device there was an ignition hood. Into this ignition hood 2435 normal cubic meters of blast furnace gas were burnt. The

ating value of the blast furnace gas was 900 calories per normal cubic meter. The sinter output in this conventional process was 75 tons per hour. The consumption of coke was 101.9 kg. per ton sinter=530,000 calories per ton sinter and the blast furnace gas consumption for the ignition was 32.4 normal cubic meters per ton sinter=29,200 calories per ton. The whole consumption was 559,200 calories.

## EXAMPLE 2

Over the same sinter band a second hood for the simultaneous application of hot gases and solid fuel was built adjoining to the ignition hood. Both the hoods together covered 35 percent of the sinter band area. The second hood was divided in three sections. According to the conventional art in the whole hood—just as in the ignition hood—a temperature of 1100° C. was maintained. Again the same steel-iron sinter mixture was used. The recycled material was the same. The coke addition, however, was reduced to 4.9 parts for 100 parts of the mixture. The consumption of gas in the heating hood including ignition hood was now 9400 normal cubic meters per hour. The quality of the sinter produced corresponded to the sinter of the Example 1. The output of the sinter band, however, decreased to 15.6 tons per sinter per hour. The consumption of coke per ton of sinter was 60.1 kg.=312,500 kilo calories; the blast furnace gas consumption was 148 normal cubic meters=133,200 kilo calories. Thus the whole consumption was 445,700 kilo calories. The consumption of calories was 20.3 percent lower than in Example 1. At the same time, however, a decrease of the output of 15.2 percent took place in comparison to Example 1.

## EXAMPLE 3

In a third test the temperature was regulated in the invention and the following hood according to the invention as follows:

|                                             | ° C. | 40 |
|---------------------------------------------|------|----|
| Temperature in the ignition hood            | 1070 | 40 |
| Temperature in the hood with the cooler gas | 650  |    |
| Temperature in the next hood                | 1050 |    |
| Temperature in the following hood           | 1100 |    |

The ore mixture again was iron ore sinter mixture the same composition as in Examples 1 and 2. Also the return material charge amounted to about 32 per-

cent. The coke addition was 5 parts of coke fines for 100 parts of ore. The blast furnace gas consumption was 9180 normal cubic meters per hour. With the regulation of temperature as described above the output of the sinter band was 74.5 tons sinter per hour. It corresponds practically to the output of Example 1. The consumption of coke fines was now 61.4 kg. per ton sinter=319,000 kilo calories per ton sinter in the same order of magnitude as in Example 2. The blast furnace gas consumption was 123.2 normal cubic meters per ton sinter=111,000 kilo calories. The whole heat consumption was 430,000 kilo calories. The consumption of the fuel was 21.3 percent lower than in Example 1. The quality of the sinter corresponded to Example 1.

Having now described the means by which the objects of the invention are obtained.

We claim:

A process for the endothermic treatment of material moving horizontally on a sinter apparatus comprising forming a bed composed of a mixture of the material and solid fuel on said sinter apparatus, drawing hot gas through the bed to ignite the solid fuel and supply additional heat to said bed and thereby form a melting zone of the material in the bed, then drawing a gas cooler than said hot gas through said melting zone in said bed in quantities sufficient to limit an increase in the width of said melting zone and to maintain a thin gas permeable zone in advance of said melting zone and below melting temperature with said cooler gas being hot enough to supply sensible heat to said sinter bed, and then drawing another hot gas at a temperature higher than said cooler gas through said bed for forming a second zone at a temperature less than that of said melting zone but greater than that of thin gas permeable zone.

35

## References Cited in the file of this patent

## UNITED STATES PATENTS

|           |           |               |
|-----------|-----------|---------------|
| 2,235,261 | Labbe     | Mar. 19, 1941 |
| 2,380,056 | Lloyd     | July 10, 1945 |
| 2,441,383 | Babb      | May 11, 1948  |
| 2,498,766 | Pettigrew | Feb. 28, 1950 |
| 2,750,274 | Lellep    | June 12, 1956 |

## FOREIGN PATENTS

|         |               |               |
|---------|---------------|---------------|
| 573,539 | Great Britain | Nov. 26, 1945 |
| 720,302 | Great Britain | Dec. 15, 1954 |

45